

## UNITED STATES PATENT OFFICE

CLIFTON TAYLOR, OF PITTSBURGH, PENNSYLVANIA, AND HERMAN L. GREENE, OF TOLEDO, OHIO, ASSIGNORS TO MOLYBDENUM CORPORATION OF AMERICA, OF PITTSBURGH, PENNSYLVANIA, A CORPORATION OF PENNSYLVANIA

## CAST-IRON ALLOY

No Drawing.

Application filed April 21, 1927. Serial No. 185,649.

The invention relates to cast iron alloys, and its object is to provide a cast iron alloy which may be easily hardened to a variable degree, and to which a very high degree of hardness may be given, and which may be more readily machined than ordinary cast iron.

In the practice of this invention ordinary cast iron, containing the usual amounts of 10 carbon and silicon, has certain amounts of nickel and molybdenum added to it, and contains no other purposely added alloying constituent. The amounts of carbon and silicon present in ordinary cast iron, as here 15 contemplated, are from about 1.0 to 4.0% carbon, and from about .5 to 2.5% silicon. To this there are added nickel from about 1.0 to about 4.0%, and molybdenum not more than about 1.0%. The alloy will of course 20 contain other constituents present as impurities and as incidental to its manufacture from commercial scrap and other materials. For example, small amounts of sulphur, phosphorus and manganese may be present 25 as impurities from the pig metal used in a cupola melt, and larger amounts of chromium, vanadium, copper, etc., may be present as constituents found in commercial scrap used also in a cupola melt.

Within the stated ranges of the purposely 30 added alloying constituents, it is preferred to use about 1.5% nickel and about .25% molybdenum. The content of carbon is preferably about 1.5% and that of silicon 35 preferably about 1.5%.

We have found that when articles made 40 from the alloy provided according to this invention are cast in permanent or other chill molds, they have a very high hardness, ranging from about 700 to 800 Brinell, and that when cast in sand or other non-chill 45 molds, they have a hardness of about 200 Brinell. Although the latter is about 50 points higher than ordinary cast iron, we have nevertheless found that the alloy has a dense close grain and that it is more readily machinable than ordinary cast iron.

Having these physical characteristics, the 50 alloy is particularly suitable for the manufacture of articles, some portions of which it

is desired to provide with hardened surfaces, and other portions of which it is desired to have relatively soft for machining and other purposes. An example of such articles is tappets for operating the valves 55 of internal combustion engines. The alloy is also particularly suitable for the manufacture of cylinder blocks and pistons for internal combustion engines in that it is very resistant to wear, has but little tendency to grow, and is readily machinable.

According to the patent statutes we have 60 explained the principle of our invention and have described what we now consider to represent its best embodiment. However, we 65 desire to have it understood that, within the scope of the appended claims, the invention may be embodied in cast iron alloys other than that specifically described.

We claim as our invention:

1. A cast iron alloy consisting of about 70 1.5% nickel, about .25% molybdenum, silicon from about .70 to about 2.5%, and carbon from about 1.5 to about 4.0%, the remainder of the alloy being iron except for 75 constituents present as impurities and as incidental to the manufacture of the alloy.

2. A cast iron alloy consisting of from 80 about 1.0 to about 4.0% nickel, a substantial and effective amount of molybdenum up to about 1.0%, silicon from about .80 to about 2.5%, and carbon from about 1.5 to about 4.0%, the remainder of the alloy being iron except for constituents present as 85 impurities and as incidental to the manufacture of the alloy.

3. A cast iron alloy consisting of about 90 1.5% nickel, about .25% molybdenum, about 1.5% silicon, and from about 1.5 to 4.0% carbon, the remainder of the alloy being iron except for constituents present as impurities and as incidental to the manufacture of 95 the alloy.

In testimony whereof, we hereunto sign our names.

CLIFTON TAYLOR.  
HERMAN L. GREENE.